

# United States Patent

Schneggenburger et al.

[15] 3,639,139

[45] Feb. 1, 1972

[54] ALUMINUM PLATING PROCESS

[72] Inventors: Roger G. Schneggenburger, Freeland; Reinhold Hellmann, Midland, both of Mich.

[73] Assignee: The Dow Chemical Company, Midland, Mich.

[22] Filed: Oct. 7, 1968

[21] Appl. No.: 765,621

[52] U.S. Cl. .... 117/37 R, 106/1, 117/47 R, 117/124 C, 117/130 R, 117/138.8 R, 117/143 B, 117/160 R, 117/212, 117/227

[51] Int. Cl. .... C23c 3/04

[58] Field of Search: 117/130, 160, 212, 227, 107.2, 117/119.8, 46, 37, 47, 124, 138.8, 143; 23/204, 205

[56] References Cited

UNITED STATES PATENTS

3,206,326 9/1965 Whaley et al. .... 117/107.2  
3,214,288 10/1965 McGraw ..... 117/130 X

|           |         |                     |           |
|-----------|---------|---------------------|-----------|
| 3,387,933 | 6/1968  | Snyder.....         | 23/204    |
| 3,453,089 | 7/1969  | Del Givdice .....   | 23/204 X  |
| 3,462,288 | 10/1969 | Schmidt et al. .... | 117/130 X |
| 2,125,827 | 8/1938  | Turkington.....     | 117/119.8 |
| 3,256,109 | 6/1966  | Berger .....        | 117/212 X |

Primary Examiner—Ralph S. Kendall

Attorney—Griswold & Burdick, William R. Norris and Bruce M. Kanuch

[57]

## ABSTRACT

A process for depositing a metallic aluminum film on a substrate material which comprises: depositing a transition metal catalyst on said substrate; depositing an aluminum hydride compound on said substrate in contact with said catalyst; contacting said treated substrate in a heated bath consisting of an inert liquid, thereby decomposing said aluminum hydride material and providing a metallic aluminum coating on said substrate; removing said aluminum coated substrate from said bath and removing said inert liquid to provide said metallic aluminum coating on the substrate.

10 Claims, No Drawings

## ALUMINUM PLATING PROCESS

## BACKGROUND

It is known that metallic aluminum may be plated from aluminum hydrides by contacting such hydrides with a substrate at or above the decomposition temperature of the aluminum hydride. Such a process usually requires relatively high temperatures to cause decomposition of the aluminum hydride and therefore cannot be used to plate aluminum onto many heat-sensitive substrates. Moreover, necessary heat is usually supplied to the reaction systems by such means as convection ovens, heat guns, radiant heat and the like. It is difficult to maintain critical temperature control when employing such heating means. Consequently the plates thus formed are not consistently of a uniform adherent nature. It would be highly desirable, therefore, to have a process which would permit the uniform plating of aluminum at relatively low temperatures.

Also, since many aluminum hydride compounds are unstable in the presence of water, it is desirable in order to prepare superior films, to decompose the hydrides in the presence of a substantially anhydrous inert atmosphere. A further desideratum of the art, therefore, is to provide a method allowing the use of water-unstable hydrides. It would, therefore, also be desirable to have a process which would permit the plating of aluminum at relatively low temperatures and to be able to control the atmosphere and temperature within predetermined critical limits. This would allow the plating of heat-sensitive substrates and improve the film characteristics of the aluminum plate produced. The present process now provides a method for preparing aluminum films on various substrates while employing lower reaction temperatures and with more precise control over the process conditions.

## SUMMARY

The present invention comprises depositing on a substrate a transition metal catalyst capable of decomposing aluminum hydrides to form metallic aluminum coatings at a relatively low temperature; depositing on said substrate in the presence of the catalyst an aluminum hydride compound; immersing said catalyst and aluminum hydride coated substrate in a heated inert liquid bath to decompose the aluminum hydride compound thereby forming a metallic aluminum coating on the substrate; removing the aluminum coated substrate from the bath and removing the excess inert liquid.

## PREFERRED EMBODIMENT

In the practice of the present invention substantially any solid material is suitable as a substrate. For example, metals such as iron, magnesium, brass and copper, polymers such as polyolefins, polyamides and polymeric fluorocarbons, glass, paper, cloth, carbon and graphite, wood, ceramics and the like can all be plated with aluminum by the process of this invention. The nature of the surface being plated determines to a large extent the brightness of the aluminum plate. In general, the use of a smooth, nonporous surface such as found on most metals and some polymer films produces a brighter plate than a relatively porous surface such as those encountered with paper or cloth. On the surfaces of some polymers such as polyethylene, polytetrafluoroethylene, acrylonitrile-butadiene-styrene terpolymers and polypropylene, it has been found that even better adhesion of the aluminum plate is achieved if the surface has been made more polar e.g., by sulfonation, corona discharge and the like, prior to plating with the aluminum. Various shaped objects may also be plated by the process such as, for example, whisker materials, reflectors, automobile trim and other decorative objects.

The term "aluminum hydride" is used herein in its broad sense and is meant to include any hydride compound which contains at least one aluminum atom to which at least one hydrogen atom is directly bonded and includes both the solvated and nonsolvated forms of those aluminum hydrides occurring in both forms. Included, therefore, are aluminum trihydride, the substituted aluminum hydrides such as those

having the empirical formula  $AlH_nX_{3-n}$  wherein X is a halogen, or —OR group or an —R group (wherein R is an alkyl, substituted alkyl, aryl or substituted aryl group) and n has a numerical value equal to or less than three. Also included are the complex aluminum hydrides such as  $LiAlH_4$ ,  $NaAlH_4$ ,  $Mg(AlH_4)_2$  and the like and complex substituted aluminum hydrides such as those having the empirical formula  $M(AlH_mX_4 - m)_a$  wherein X has the definition given above. m has a numerical value equal to or less than four and M is a metal or mixture of metals, preferably an alkali or alkaline earth metal and a has a numerical value equal to the valence of M. Of particular utility are the relatively simple aluminum hydrides containing at least two hydrogen atoms attached to the aluminum, e.g.,  $AlH_3$ ,  $AlH_2Br$ ,  $LiAlH_4$ , and the like. Mixtures of the various aluminum hydrides may also be employed.

It is usually desirable for ease of application to employ the aluminum hydride in solvated form. Compounds known to solvate or form complexes with the aluminum hydrides include ethers and other oxygen-containing organic compounds, and compounds containing a functional group such as a divalent sulfur atom, or trivalent nitrogen or trivalent phosphorous atom which is capable of allowing the solvation of an aluminum hydride with such compound. It is usually preferred that the solvate be an etherate and a wide variety of ethers containing from about two to about 20 carbon atoms are suitable. Usually the lower aliphatic ethers such as ethyl, propyl, or butyl ethers are employed but those containing an aromatic group such as methylphenyl ether, ethylphenyl ethers, propylphenyl ether or the alicyclic ethers such as tetrahydrofuran and the like may be employed.

In general, to achieve ease and uniformity of application of the aluminum hydride compound, any solvent or mixture of solvents or suspending agents for the aluminum hydride may be employed which will not react with the aluminum hydride beyond the formation of a complex or solvate. Suitable solvents include aromatic hydrocarbons such as benzene, toluene and xylene, aliphatic hydrocarbons such as hexane, ethers, tertiary amines and the like.

If desired, such aluminum hydrides may be prepared in situ simultaneously with the plating step by employing aluminum hydride-forming reactants such as mixtures of lithium aluminum hydride and aluminum chloride, or sodium aluminum hydride and aluminum bromide, or the like. The presence of a metal halide such as  $LiCl$ ,  $MgCl_2$  or  $AlCl_3$  together with the aluminum hydride is not detrimental to the plating reaction.

In order to produce decomposition of the aluminum hydrides below their normal decomposition temperatures and to cause the aluminum thus produced to form a coating or plate on the substrate, it is necessary to contact the aluminum hydride with certain transition metal decomposition catalysts. Transition metal decomposition catalysts useful herein are compounds of the metals occurring in Groups IVb and Vb of the periodic table. In instances where the catalyst is applied to the substrate in a solvent, it is preferable that the metal be in the form of a compound which is soluble to the extent of at least  $1 \times 10^{-6}$  weight percent of the solvent employed. For example, such compounds as  $ZrCl_4$ ,  $NbCl_5$ ,  $VOCl_2$ ,  $VOCl_3$ ,  $TiCl_4 \cdot 2(C_2H_5)_2O$ ,  $TiCl_4$ ,  $TiBr_4$ ,  $VCl_4$ ,  $Ti(OC_2H_5)_2Cl_2$ ,  $TiCl_2(i-OC_3H_7)_2$ ,  $TiCl_2 \cdot 2[(C_2H_5)_2O]$ ,  $Ti(BH_4)_3[(C_2H_5)_2O]$  have proved effective. Some of the transition metal catalysts defined herein have a more pronounced effect than others in lowering the decomposition temperature of the aluminum hydride. The chlorides, bromides and oxychlorides of titanium, niobium, vanadium and zirconium generally seem to be more effective than the other compounds of Group IVb and Vb transition metals and  $TiCl_4$  has been found particularly effective in achieving lower temperature decomposition of the aluminum hydrides and plating of the aluminum thus produced. If the defined catalysts are not employed, undesirably high temperatures are required to produce decomposition of the aluminum hydride. At such elevated temperatures, even when decomposition is achieved, there is usually no aluminum coating or plate formed thereby.

The transition metal decomposition catalyst is preferably applied to the substrate prior to contact with the aluminum hydride. Such decomposition catalyst may be applied to the substrate directly as a finely divided solid, as a liquid solution or suspension or, where the nature of the catalyst and the substrate permit, deposited by vapor deposition. Preferably, however, the substrate is contacted with a sufficient quantity of a relatively dilute solution of the catalyst to wet the surface of the substrate. The solvent for the catalyst is then removed, e.g., by evaporation, leaving the catalyst substantially uniformly dispersed over the surface to be plated. Catalyst solutions at least about  $1 \times 10^{-6}$  weight percent in decomposition catalyst, and preferably in concentrations of from about  $5 \times 10^{-6}$  to about 100 weight percent of catalyst when applied to the substrate provide sufficient catalyst to achieve plating of aluminum from an aluminum hydride at a significantly lower temperature than is possible where no catalyst is employed. It has been found that uniformity of distribution of the catalyst on the substrate has a significant effect on both the uniformity and thickness of the aluminum plate. It is, therefore, desirable to apply the catalyst to the substrate in a manner which will assure relatively uniform distribution.

For substrates, such as magnesium metal and some solid polymers, having surface characteristics making uniform distribution of a catalyst solution or aluminum hydride difficult to achieve, it has been found advantageous to add to such solution a small amount, e.g., from about 0.0001 to about 5.0 weight percent, of a wetting agent. Suitable wetting agents include, for example, stearates such as sodium or aluminum stearate or aluminum alkoxides such as aluminum isopropoxide.

Solvents for the transition metal decomposition catalysts are those normally liquid materials in which the catalyst is soluble to at least the extent of  $1 \times 10^{-6}$  weight percent, which will not adversely effect the substrate and which will not change the anion of the catalyst sufficiently to render it insoluble. Suitable solvents include nonreactive solvents such as benzene, hexane, and halogenated hydrocarbons, reactive solvents such as alcohols, aldehydes, ketones, mercaptans, carboxylic acids and mineral acids, and coordinating solvents such as ethers, nitriles, amides and amines.

By application of the transition metal decomposition catalyst to only selected areas of the substrate, it is possible to form an aluminum plate only on such selected areas. In this manner, ornamental designs, outlines, printed circuits and the like may be produced. Likewise, all or a portion of a selected substrate may be coated or plated with aluminum to enhance the ability of such surface to adhere to other materials. Of particular utility is the aluminum coating of glass, ceramic, metal or polymer surfaces to enhance their bonding to adhesive polymers and copolymers such as the copolymers of ethylene and acrylic acid.

Once the desired form and quantity of decomposition catalyst is applied to the substrate, the catalyzed substrate surface is contacted with a suitable form of aluminum hydride. In general, it is desirable to apply the aluminum hydride as a solution or suspension from 0.1 to 1.0 molar or more in aluminum hydride which may be applied by dipping, spraying or other suitable means. However, good results are also achieved by contacting the catalyzed substrate surface with a finely divided solid aluminum hydride.

The solvent for the aluminum hydride compound is usually evaporated and the so-treated substrate is then immersed in the hot inert liquid bath.

The inert liquid bath can consist of any substance which is a liquid at elevated temperatures, usually at temperatures of from 50° to about 200° C. and which is substantially inert to aluminum hydride and the particular substrate employed. The bath should be substantially anhydrous, i.e., usually containing less than about 20 parts per million of water, due to the sensitivity of most aluminum hydrides to moisture. Likewise, the application of the aluminum hydride compound to the substrate material should be conducted in a substantially an-

hydrous inert atmosphere for best results. Suitable materials which can be employed for the inert liquid bath consist of, for example, organic substances such as naphtha, ethylbutylbenzene, ethylbenzene, diphenyl ether, octadecane, xylene and other like materials. Other inert aliphatic, aromatic and ether compounds which are liquid at the indicated temperature range can be employed. The inert liquid bath, however, should not be prepared from compounds which contain active species such as alcohols, ketones, aldehydes, esters, acids and unsaturated aliphatics since the aluminum plate which develops will be dark, uneven and the substrate will contain unplated areas. It has also been found convenient, although not essential to employ an inert liquid bath which boils in the range of about 100° to about 140° C. Such a bath will allow the application of heat for producing the aluminum plate, and evaporate quickly to provide an even adherent aluminum plate on the substrate. Higher boiling inert liquids can be removed, for example, by wiping or draining the coated substrate material.

As indicated previously the bath should usually be maintained at a temperature of about 50° to about 200° C. A temperature of from about 100° to about 150° C. is usually preferred. The actual decomposition temperature of aluminum hydride compounds catalyzed by the transition metal catalysts defined herein will vary depending on the particular aluminum hydride compound employed, upon the catalyst used and to some extent, upon the catalyst concentration. Such decomposition temperatures will, however, be substantially lower than those required where no catalyst is present.

The present process can be run as a continuous operation for the coating of various shaped objects such as films, webs, paper and the like. Also, it may be employed to coat various other objects such as whisker materials, beads, powders, various irregularly shaped forms of reflectors for lights, piping and the like. Thus, by employing the transition metal catalyst and inert liquid bath, aluminum coatings can be applied to heat-sensitive substrates. Likewise, more precise control over the process conditions can be had by use of the bath with the result that aluminum coatings of superior quality can be prepared.

The following examples will facilitate a more complete understanding of the present invention.

45

#### EXAMPLE 1

Several irregularly shaped metal objects were first coated with a metal catalyst consisting of  $TiCl_4$  dissolved in an inert solvent consisting of diethyl ether and the solvent evaporated. Next, an  $AlH_3$  solution consisting of 0.25 molar  $AlH_3$  in diethyl ether was applied to the samples and the solvent again evaporated. A substantially water-free bath consisting of naphtha was then prepared and heated to a temperature of about 130°-140° C. The objects were submerged in the bath for about 5 to 10 seconds whereupon a shiny adherent uniform aluminum film was deposited onto the objects. The objects were removed from the baths and the excess naphtha allowed to evaporate from the surface of the aluminum plate.

60

#### EXAMPLE 2

In a manner similar to that described in example 1, 2 mil thick Mylar brand polyester film samples were treated with the catalyst and  $AlH_3$  solution as described in example 1 and then placed in several different heated baths. All the baths were heated to about 130° C. The baths employed consisted of an eutectic mixture of diphenyl and diphenyl oxide; ethyl butyl benzene; naphtha and a 200 centistoke methyl end blocked dimethylpolysiloxane. All the samples were plated with a shiny adherent Al film.

Various modifications may be made in the present invention without departing from the spirit or scope thereof for it is understood that we are limited only as defined in the appended claims.

75 What is claimed is:

1. In the process of plating metallic aluminum onto a substrate wherein coating a substrate with an aluminum hydride compound in the presence of an aluminum hydride decomposition catalyst comprising a compound selected from the group consisting of compounds of the metals of Groups IVb and Vb of the periodic table, and subjecting the coated substrate to sufficient energy to plate said aluminum onto the substrate, the improvement which comprises:

- a. contacting said substrate with an inert liquid bath, maintained at a sufficient temperature to decompose said aluminum hydride compound thereby depositing metallic aluminum on said substrate;
- b. removing the aluminum coated substrate from said bath;
- c. removing excess inert liquid from said aluminum plated substrate material.

2. The process as defined in claim 1 wherein said aluminum hydride compound is a solvated aluminum hydride compound.

3. The process as defined in claim 1 wherein said decomposition catalyst and said aluminum hydride compound are applied to said substrate material as liquid dispersions containing said decomposition catalysts and said aluminum hydride compounds.

4. The process as defined in claim 3 wherein said liquid dispersions contain a surface wetting agent.

5. The process as defined in claim 1 wherein said inert bath consists of a substantially anhydrous material which is a liquid

at a temperature of from about 50° to 200° C., and is further characterized as being nonreactive with said aluminum hydride compounds, said catalyst compounds and said substrate material.

6. The process as defined in claim 1 wherein said inert bath consists of a substantially anhydrous material which is a liquid at a temperature of from about 100° to 140° C. and is further characterized as being nonreactive with said aluminum hydride compound said catalyst compound and said substrate material.

7. The process as defined in claim 1 wherein said inert bath is maintained at a temperature of from about 50° to 200° C.

8. The process as defined in claim 1 wherein said decomposition catalyst is applied to the substrate as a solution containing at least  $1 \times 10^{-6}$  weight percent catalyst and the aluminum hydride compound is applied to the catalyst-treated substrate in a liquid dispersion containing at least 0.0001 weight percent of said aluminum hydride compound.

9. The process as defined in claim 1 wherein said substrate is a shaped object of a material selected from the group consisting of organic polymers, glasses, ceramics, metals and cellulose fibers.

10. The process as defined in claim 1 wherein said decomposition catalyst is applied to only a portion of the substrate to thereby produce a metallic aluminum design.

\* \* \* \* \*

30

35

40

45

50

55

60

65

70

75

UNITED STATES PATENT OFFICE  
CERTIFICATE OF CORRECTIONPatent No. 3,639,139 Dated 1 February 1972Inventor(s) Roger G. Schneggenburger and Reinhold Hellmann

It is certified that error appears in the above-identified patent and that said Letters Patent are hereby corrected as shown below:

Column 2, line 60, add a bracket so it reads:  $--\text{TiCl}_4 \cdot 2[(\text{C}_2\text{H}_5)_2\text{O}]$ ,

line 61, add  $--2--$  so it reads:  $\text{Ti}(\text{BH}_4)_3 \cdot 2[(\text{C}_2\text{H}_5)_2\text{O}]$ .

Column 3, line 14, change " $5 \times 10^{-7}$ " to  $-- 5 \times 10^{-5} --$ .

Signed and sealed this 8th day of August 1972.

(SEAL)

Attest:

EDWARD M. FLETCHER, JR.  
Attesting OfficerROBERT GOTTSCHALK  
Commissioner of Patents